

April 25, 1933.

H. B. LIND

1,905,565

PRODUCTION OF SIGNS, DECORATIONS, AND THE LIKE

Filed Oct. 22, 1929



Fig - I



Fig - II

Howard B. Lind  
INVENTOR.  
BY *John Marshall*

ATTORNEY.

## UNITED STATES PATENT OFFICE

HOWARD B. LIND, OF TOLEDO, OHIO, ASSIGNOR TO THE TOLEDO PORCELAIN ENAMEL PRODUCTS COMPANY, OF TOLEDO, OHIO, A CORPORATION OF OHIO

## PRODUCTION OF SIGNS, DECORATIONS, AND THE LIKE

Application filed October 22, 1929. Serial No. 401,615.

This invention relates to the production of signs, decorations or other decorative articles by stenciling, the chief object being to enable vitreous i. e. so called porcelain 5 enamel metal signs and the like to be manufactured commercially in large numbers in a rapid, inexpensive and simple manner.

Hitherto the commercial production of vitreous enamel metal signs, particularly signs 10 with complicated or multi-colored designs or lettering thereon, has been limited owing to the many operations and great labor and expense involved in the method of production hitherto employed. The drawback and 15 limitations to printing methods with the aid of a litho-stone or zinc plate, the aerographing method, and the "brushing out" method are well known in the trade.

According to the present invention vitreous 20 enamel metal signs or other decorative articles are produced by preparing an enameling composition or paint of suitable consistency and drying characteristics, applying the composition to a vitreous surface 25 to be decorated by means of a screen or stencil of silk or other meshed material having permeable and impermeable portions, and finally heating the article so treated to a 30 temperature sufficient to cause fusion of the vitreous surface. In the preparation of the 35 paint or composition a finely ground mineral color is used as the body or base which is mixed with oil and worked up to a suitable consistency to pass through the meshes of the stencil employed.

The fineness of the powdered materials should be as great as is necessary to enable the composition to pass through the meshes of the stencil and the materials should therefore 40 be capable in their dry unmixed state of passing through a screen of slightly finer mesh.

In working up the powdered color mixture into a suitable pasty mass a liquid must be 45 used that will not permit of too rapid drying and yet can eventually be dried completely without causing the surface to be spoiled by bubbles or otherwise when the article is subjected to the "enamel fusing" temperature. 50 I have found that liquid of an oily

character should be used. The pasty composition is effectively and simply applied by pressing it through the meshes of the stencil by means of a squeegee. When articles are enameled by the so-called wet process 55 the frit is mixed with water, sprayed upon the articles and the water evaporated off, leaving the metallic base coated with a powdery layer of frit which is sufficiently adherent to permit decoration by my process if 60 care is exercised in application of the decorative material. By applying the decorative material to the unfused frit, one firing is avoided. Usually, however, it will be found more advantageous to fuse the frit 65 before applying the decorative material. After stenciling the porcelain enamel on the metal sheets as above described I may first heat them sufficiently to dry out the oily medium and then heat them in a muffle furnace or otherwise to a temperature sufficient 70 high to cause fusion of the vitreous enamel background with the colored composition applied through the stencil, for example from say about 600° to 1000° C. depending upon the nature of the composition. I thereby obtain real vitreous enamel sheet metal advertising signs or the like.

The usual method of placing the lettering or other designs on porcelain enamel signs is to first apply a coat of dark enamel to the metal, fuse it, then apply a coat of light colored enamel and, before fusing, wipe away the lettering or design by means of stencils. When the light colored enamel 80 is fused, the dark lettering or design appears as sunken or depressed. My process obtains a similar result. For some reason unknown to me but which I suppose results from a lowering of the surface tension of the fused 85 enamel where the oily mixture has been applied, the enamel appears to partially withdraw when it is fused, so that the letter or design is depressed and its appearance is substantially the same as though it had been 90 made by wiping away the upper enamel before fusing.

The result obtained by my process is illustrated in the accompanying drawing, in which Figure I is a front elevation of an 100

enameled metal plate 1 with the letter N 2 produced thereon by the process of my invention, the color of the enameled field 3 being white and the color of the letter N 5 being red; and

Figure II is a sectional view on an enlarged scale taken on the line II—II of Figure I, the depth of the porcelain enamel and the depth of the red color and the depression 10 in which the color lies being exaggerated.

I am aware of the process described in Reissue Patent No. 16,048, but the process developed by me differs from that described 15 in the said reissue patent in that I avoid the use of frit in the coloring composition and also in that I obtain a different and superior result, one substantially the same as that produced by the very much more expensive 20 process of wiping away the upper coat of enamel before fusing.

The embodiment of my invention herein described is to be regarded as illustrative only, and it is to be understood that the invention 25 is susceptible to variation, modification and change within the spirit and scope of the subjoined claims.

Having described my invention, I claim:

1. The method of producing designs upon 30 porcelain enamel which consists in taking a pasty composition of mineral coloring matter and an oily carrier containing no frit capable of causing a change in the depth of porcelain enamel to which it is applied, 35 applying the said composition to a layer of porcelain enamel material upon a metallic object, and subjecting the enamel so treated to fusing.

2. The method of producing designs upon 40 porcelain enamel which consists in taking a pasty composition of mineral coloring matter and an oily carrier containing no frit capable of causing a change in the depth of porcelain enamel to which it is applied, 45 applying the said composition to a layer of porcelain enamel material upon a metallic object by pressing the composition of coloring matter through a fine mesh stencil, and subjecting the enamel so treated to fusing.

50 HOWARD B. LIND.